

## UNITED STATES PATENT OFFICE.

MICHAEL G. CORSON, OF JACKSON HEIGHTS, NEW YORK, ASSIGNOR TO ELECTRO METALLURGICAL COMPANY, A CORPORATION OF WEST VIRGINIA.

## CORROSION-RESISTANT ALLOYS.

No Drawing.

Application filed April 13, 1926. Serial No. 101,813.

The invention relates to copper-manganese alloys and comprises a group of compositions of this class which are highly resistant to attack by corrosive agents, such for example as the inorganic acids.

I have discovered that the property of corrosion-resistance is developed to a remarkable degree in copper-manganese alloys when the manganese content is between 35% and 55%. Alloys of these two metals containing up to 20% of manganese have been used industrially, and other alloys of the series with higher manganese have been prepared in the laboratory; but the former alloys show little resistance to corrosion and it has not been observed that any alloys of the latter group were superior in this respect.

The ability of the alloys of the invention to resist corrosion is apparently due to the relationship between the manganese and copper contents, and there are several other elements which may be present in moderate amounts without important effect on the properties of the alloy. Among these there may be mentioned tin, zinc, nickel and iron. The manganese used in making the alloy may be the product of reduction by carbon, silicon, or aluminum. If carbon-reduced metal carrying more than about 0.5% of carbon is used, the final alloy is unable to dissolve the whole of the carbon thus introduced. Usually about 0.2% to 0.3% of carbon will be found in the finished alloy under these conditions, and any excess carbon will eliminate itself by rising to the surface of the melt. Silicon, if present in too great quantity, is somewhat detrimental to the corrosion-resistance of the alloy and injures its working properties to a great extent. Aluminothermic manganese is quite suitable for the manufacture of said alloys.

The binary copper-manganese alloys containing 35% to 55% of manganese appear to be solid solutions, at least when they are quenched from 850° C. Alloys made in practicing the invention will usually not be strictly binary in character as other elements will be intentionally added or will be introduced through the use of the impure commercial grades of raw materials. Measures should then be adopted to insure homogeneity in the alloy.

Quenching the alloy from a temperature between 750° C. and its melting point, acts to prevent or diminish the precipitation of impurities from solid solution and thus produces a material better adapted to resist corrosion. Such treatment also puts the alloy into the optimum condition for cold work. After cold work, such as rolling, the alloy is preferably reheated to a temperature above 750° C. and annealed at this temperature to remove all strains which as is known are prejudicial to resistance to corrosion. After the annealing the alloy may be cooled slowly or quenched, the latter procedure being preferable in that it tends to insure homogeneity in the alloy.

The following figures illustrate the mechanical properties attainable with alloys according to the invention:

|                             | Cold rolled, 75% reduction.        | Annealed at 850° C., then quenched. | 75 |
|-----------------------------|------------------------------------|-------------------------------------|----|
| Tensile strength.....       | 125,000 lb./in. <sup>2</sup> ..... | 85,000 lb./in. <sup>2</sup> .....   |    |
| Yield point.....            | 65,000 " ".....                    | 25,000 " ".....                     |    |
| Elongation in 2 inches..... | 3%.....                            | 30%.....                            |    |

The composition preferred for most purposes is one containing about 42% of manganese.

I claim:

1. An article of manufacture adapted to resist corrosion by inorganic acids, composed of an alloy containing 35% to 55% manganese with the balance principally copper.

2. An article of manufacture adapted to resist corrosion by inorganic acids, composed of an alloy containing about 42% of manganese with the balance principally copper.

3. Process of preparing articles resistant to corrosion which comprises forming the article from a copper-manganese alloy containing 35% to 55% manganese and annealing the article at a temperature above 750° C.

4. Process of preparing articles resistant to corrosion which comprises forming the article from a copper-manganese alloy containing 35% to 55% manganese, annealing the article at a temperature above 750° C., and then quenching.

In testimony whereof, I affix my signature.

MICHAEL G. CORSON.